

Aug. 20, 1929.

A. KADOW

1,725,144

# PROCESS AND APPARATUS FOR CASTING HOLLOW ARTICLES

Filed March 15, 1926

4 Sheets-Sheet 1



Inventor  
**AUGUST KADOW**

Owen & Owen

Attorneys

Aug. 20, 1929.

A. KADOW

1,725,144

## PROCESS AND APPARATUS FOR CASTING HOLLOW ARTICLES

Filed March 15, 1926

4 Sheets-Sheet 2



Inventor  
**AUGUST KADOW**

By Owen & Owen

Attorneys

Aug. 20, 1929.

A. KADOW

1,725,144

PROCESS AND APPARATUS FOR CASTING HOLLOW ARTICLES

Filed March 15, 1926

4 Sheets-Sheet 3



Inventor  
**AUGUST KADOW**

834

Owen & Owen

Attorneys

Aug. 20, 1929.

A. KADOW

1,725,144

# PROCESS AND APPARATUS FOR CASTING HOLLOW ARTICLES

Filed March 15, 1926

4 Sheets-Sheet 4



Inventor

AUGUST KADOW

३५

Owen & Owen

Attorneys

## UNITED STATES PATENT OFFICE.

AUGUST KADOW, OF TOLEDO, OHIO, ASSIGNOR OF ONE-HALF TO WILBUR OWEN  
AND CHARLES W. OWEN, OF TOLEDO, OHIO.

## PROCESS AND APPARATUS FOR CASTING HOLLOW ARTICLES.

Application filed March 15, 1926. Serial No. 94,713.

My invention relates to a method of and apparatus for casting metal, and more particularly to casting hollow articles without the use of a core.

5 The object of my invention is to provide a method and apparatus whereby hollow metal articles may be made rapidly and accurately.

In general, my method consists in filling 10 a mold with liquid metal and allowing the interior liquid metal to run out of the mold after a shell of solidified metal has formed against the inside of the mold. In order to increase the uniformity of thickness of the 15 walls and the smoothness of the interior of the article, I introduce air into the interior of the mold to displace the liquid metal rapidly and with certainty. When necessary for a smooth job, additional air pressure is 20 applied to the interior of the article after it is emptied of liquid metal.

My apparatus consists of devices suitable 25 for carrying out my method. The details and minor objects of my invention will appear as the description proceeds.

In the accompanying drawings forming a part of this specification, Figure 1 is a vertical longitudinal section of one form of my apparatus, parts being shown in elevation; 30 Fig. 2 is a section on line 2-2 of Fig. 1; Fig. 3 is a section on the line 3-3, Fig. 1, showing the greater part of the apparatus in plan; Fig. 4 is a section of the final blow-head, showing the mouth of the mold in operating position; and Figs. 5 to 8 are sections showing the relation of the mold to the metal during successive stages of the casting process. Fig. 9 is a view, partially in section and with parts broken away, showing 35 a different form of mold; Fig. 10 is an elevation of the inside of one half of the mold shown in Fig. 9; Fig. 11 is a section on line 11-11 of Fig. 9, and Fig. 12 is a perspective of the article cast in the mold 40 shown in Figs. 9 to 11.

A pedestal 10 has a collar 11 vertically adjustable thereon and rotatable thereabout. A horizontal beam 12 extends from one side of collar 11 and carries a sleeve 13 having 45 a depending pin 14. Mold-supporting arms 15 have hinge lugs 16 mounted on pins 14, and a collar 17, fastened on the lower end of pivot pin 14 by means of a pin 18, retains

the lugs on the pivot. A mold-half 19 is mounted on one end of each of the mold- 55 supporting arms.

A longitudinal frame-member 20 is attached to sleeve 13. One end of frame-member 20 is provided with a handle 21 by means of which its position and movements may 60 be controlled.

A mold-operating handle 22 is mounted upon a vertical pivot pin 23 suitably held in frame-member 20. The rear ends of arms 15 are connected by links 24 to a pin 25 65 which, in turn, is connected by a link-bolt 26 to the front end of handle 22. Bolt 26 is surrounded by a spring 27 which normally presses the bolt forward until nuts 28 on the end of the bolt contact handle 22. 70 Pin 25 has a head 29 moving in a guideway 30 in frame-member 20, so that pin 25, and consequently the center of the mold, is held in the central longitudinal line of the frame-member. 75

The mold-sections have their meeting faces hollowed out to form a mold cavity 31 and grooved to form vacuum passages 32. Preferably, the molds are ground at 33, between the mold cavity and the vacuum grooves, so 80 as to form a very thin slit through which air passes from the mold cavity to the vacuum grooves, but which is so narrow that liquid metal does not pass through it.

The mold shown is intended to form a 85 threaded article, and therefore the interior of the mold cavity is threaded at 34. I prefer not to grind away the walls for an air passage at any point where threads occur, as there is likely to be a slight fin of metal 90 left on the article along the line of any such air passage.

A vacuum chest 35 is carried on the frame above the mold. Air is exhausted from the chest through a pipe 36 leading to any means 95 suitable for accomplishing that purpose. The passage between the vacuum grooves in the mold and the vacuum chest is controlled by a valve 37 having a stem 38 and normally closed by a spring 39. 100

A valve operating bell-crank lever is pivoted to the frame at 40 and has one arm 41 in position to contact stem 38, while its other arm 42 is connected by a link 43 to a lever 44 pivoted at 45 on the frame. A cam 105 46 on the upper end of pin 23 is adapted

to contact lever 44 and open valve 37 when handle 22 is moved to the position in which it is shown in Figs. 1 and 3.

5 A crucible 47 in suitable relation to pedestal 10, has molten metal 48 therein. An air nozzle 49 projects above the normal level of the metal in the crucible. A valve 50 in the end of the nozzle is normally closed by a weight 51 attached to its stem. Weight 10 51 operates within an air chest 52 from which the nozzle rises.

5 A pipe 53 leads from a suitable air valve 54 to air chest 52. Air valve 54 is normally closed by a spring 55, but has a stem 56 extending into the path of a lever 57 pivoted at 58 to a lug 59 connected to the valve casting. A handle 60, pivoted at 61 to one of the mold-supporting arms, has a roller 62 in position to be swung against lever 57 to 20 open the valve. Stops 63 and 64 limit the movement of handle 60.

25 A blow-head 65 is suitably positioned on the crucible support beneath the line of travel of the mold as it is swung about pedestal 10. An air pipe 66, which may be a branch of the pipe leading to valve 56, conducts air into an air chamber 67. A sleeve 68 is mounted for vertical reciprocation about the air chamber, and is normally 30 raised by a spring 69.

35 A valve 70 controls the escape of air from chamber 67. The valve has a stem 71 connected by a spider 72 to sleeve 68, so that the valve is normally seated when sleeve 68 is raised by spring 69. A gasket 73 is provided on the upper surface of sleeve 68. When the mouth of the mold is rested on the gasket, as shown in Fig. 4, the sleeve and valve are depressed and air enters the mold 40 from chamber 67.

45 Sleeve 13 is adjustably positioned on beam 12 by means of collars 74 which are secured in adjusted position by set screws 75. The beam, in turn, may be secured in adjusted position by means of a set screw 76 which passes through socket-arm 77 which projects from collar 11 to receive the end of beam 12.

50 In the operation of the device, starting with crucible 47 filled with molten metal to a level 78, somewhat above chamber 52, the mold is closed by handle 22, and the frame is swung about pedestal 10 and then tilted about beam 12 to bring the bottom inlet of the mold in contact with the molten metal.

55 It may be seen, by inspecting Fig. 3, that the mold is closed before handle 22 reaches the position in which it is shown in that figure. In fact, the mold is completely closed before cam 46 actuates lever 44 to 60 open valve 37. The handle is moved to the point where the mold is closed before the mold contacts the molten metal, and thereafter the handle is moved to the position

in which it is shown in Fig. 3, thereby further compressing spring 27 and opening valve 37.

65 When valve 37 is opened, air is exhausted from vacuum channels 32 and from mold cavity 31 through slits 33 into the vacuum channels. Thereupon atmospheric pressure 70 drives the molten metal into the mold. It is desirable to close the mold before it is dipped in the metal, to avoid entrance of the metal between the faces of the mold, and it is preferable to open the vacuum valve 75 only after the mold is dipped, so as to avoid a useless draft of air through the mold. The use of one handle which may be moved a certain amount to close the mold and a further amount to open the vacuum 80 valve enables the opening of the valve immediately after the mold contacts the metal without any shifting of the operator's hand from one handle to another.

85 When metal rushes in to fill the mold, as shown in Fig. 6, the portion of the metal in contact with the comparatively cool wall of the mold immediately solidifies and forms a metal shell 79 on the inside of the mold. After the mold is filled, it is raised and the 90 metal in the interior of the shell runs out.

95 Where the inlet is of sufficient size, air bubbles will enter through the inlet and allow the molten metal to run out when the mold is lifted above the level of the molten bath; but the outflow is slightly irregular in such a case, and the inrushing air moving in the opposite direction from the out-flowing metal is likely to spray metal onto the inside of the shell and roughen the 100 interior of the shell. Air nozzle 49 is used to overcome this difficulty.

105 Weight 51 holds valve 50 seated while the mold is being filled, thus preventing the entrance of air into the mold through the nozzle. After the mold is filled, valve 54 is opened, admitting air under sufficient pressure to raise valve 50 and weight 51. Air then enters space 80. As soon as air enters the upper end of the mold, the molten metal begins to flow out by gravity, and this flow may be hastened to any desired extent 110 by increasing the air pressure. In this way the in-coming air does not have to bubble through the out-flowing metal, but, as will 115 be readily seen from Fig. 7, the air enters above the metal and drives it out quickly and evenly, so as to leave the shell with a smooth interior.

120 When the bulk of the metal has been driven out, the mold is raised to the position in which it is shown in Fig. 8. There may be a small fin 81 extending downward from the mouth of shell 79, but the shell at this 125 stage may be considered a substantially finished hollow metal article, and may be

removed from the mold immediately, if desired, and the process may be repeated to produce another article.

In order to smooth out any possible blisters or other imperfections in the interior of the cast shell, it is sometimes desirable to introduce air under pressure after the liquid metal has been removed. Blow-head 65 is provided for this purpose, and it will be readily understood that the mold with the article therein may be swung over the blow-head applied thereto in the manner shown in Fig. 4, and air pressure applied to the interior of the article.

With some kinds of metal at certain temperatures and with articles of certain shapes, there is a tendency, when the molten metal is emptied out, for a film thereof to adhere to the under side of a surface of the solidified shell and to gather in drops thereon before solidifying. It will be readily seen that this might happen on surface 82 at the top of space 80 shown in Fig. 7. If the mold is tilted to a position like that shown in Fig. 8, this surface is moved out of the horizontal plane so that, if any film adheres thereto in sufficient quantity to flow in any direction over the surface, it will flow evenly towards the lower side and will not gather in drops or seriously roughen the interior of the article. My process, therefore, includes the tilting of the mold so that no interior surface of the shell is horizontal during the emptying step, when this is found necessary to avoid the gathering of the metal in roughening drops.

If air is trapped in chamber 52 and pipe 53 under the extreme pressure which allows valve 50 to close, reduction of pressure in the mold below atmospheric allows this air under pressure to raise the valve and enter the mold. If the nozzle is sufficiently near the top of the mold, any air passing out of the nozzle may be exhausted before the metal rises above the nozzle, and under such circumstances valve 50 might even be omitted entirely. But ordinarily I prefer to use the valve, and to provide against trapping air under pressure. For this purpose, stem 56 of valve 54 is made hollow, as shown at 83 on Fig. 1, with an inlet hole 84 and an outlet hole 85. Preferably, outlet hole 85 is in such a position that when valve 54 is closed, as shown in Fig. 1, the hole is above the valve casing and acts as a vent, relieving the pressure in pipe 53 and chamber 52, but when the valve stem is depressed to open valve 54, outlet hole 85 is sealed, and so does not interfere with forcing air under pressure through nozzle 49.

The nozzle must be kept heated in order to avoid solidifying of metal about the nozzle. Conduction of heat from the portion beneath the surface of the molten metal, together with the passage of air heated in pipe

53 and chamber 52, may heat the nozzle sufficiently for this purpose, or additional heating means may be provided, or pipe 53 may be oscillated at one of its joints to immerse the nozzle between molding operations.

Of course, the air entering through pipe 53, chamber 52 and nozzle 49 is heated to about the temperature of the bath, and this is an advantage, as it prevents chilling irregularly arranged portions of metal on the interior of the shell and aids in remelting any protruding portions and smoothing the interior of the shell. Ordinarily the air thus heated is hot enough to accomplish the desired results, but, if necessary, additional heating means may be used.

The compressed air used must be free from impurities which will injure the metal within the article, and if the metal and the article being produced are of such character that heated pure air has injurious effects, another gas or gases may be selected which will avoid any injury to the hot metal.

The thickness of the solidified shell depends upon the character of the metal being cast, the temperature of the bath, the temperature of the mold and the character of its surface where it contacts the molten metal, and the length of time the molten metal remains in the mold. If the product is too thin, the bath or the mold or both may be cooled or the molten metal may be retained in the mold for a longer time. If the product is too thick, the molten metal may be discharged more quickly, the temperature of the bath or the mold or both may be raised or the interior of the mold may be coated with a non-conducting material.

The molten metal remains in contact with the lower part of the mold longer than with the upper part, and so the upper part needs to be cooler in order to obtain an even thickness in the walls of the product. Normally, the greater heating of the mold by contact with the bath and longer retention of the molten metal within it results in proper difference in temperature between the bottom and top of the mold to secure substantially even thickness in the walls of the product. Where conditions warrant, any desired portion of the mold may be artificially cooled or separately heated either to produce desired uniformity in the product or increase or decrease the thickness of the product at desired points. Where desired, a portion only of the mold may be coated with non-conducting material to reduce the thickness of the wall in the corresponding portion of the product.

It will be understood that the metal, passing the lower end of the mold as the mold is filled, heats the lower end of the mold to a higher temperature than the upper end of the mold. Therefore, if the metal remains

in contact with all portions of the wall of the mold the same length of time, the shell solidified against the mold wall would be thinner at the bottom. However, the metal contacts the lower end of the mold first, and the liquid metal is in contact with the inside of the shell at the lower end of the mold last. This normally counterbalances the heating tendency mentioned, and results in 10 a shell of substantially even thickness. However, the discharge of the metal could be so hastened as to result in a shell thinner at the lower end of the mold; or the discharge could be sufficiently slow to allow a 15 thicker shell to form at the bottom, and it is possible to even stop the discharge for a time at any desired point in order to increase the thickness of the wall below that point.

In Figs. 9 to 11 there is shown a modified device suitable for forming a head such 20 as shown in Fig. 12. In this device there is shown a mold '19' supported and operated in substantially the same way as mold 19, except for features described below.

25 The two halves of the mold are constructed somewhat differently, mold half 86 being modified merely by having its cavity shaped to conform to the back of the desired head, including the back of the ears, while half 30 87 is shaped to form the front half of the head, and is provided with means for introducing air into the mold through the ear-forming cavities.

Carried on the mold frame there is a valve 35 casing 88 into which air is introduced through pipe 89, leading from any suitable source of air under pressure. Flow of air through the valve casing is controlled by a valve 90 normally closed by a spring 91. 40 The valve has a stem 92 projecting in the path of member 93 of an operating handle 94, by which the valve may be opened when desired.

A pipe 95 having a flexible portion 96 45 leads from valve casing 88 to mold half 87.

Mold half 87 is provided with projections 97 adapted to form the hollows in the ears. The construction for the two ears is the same, and so but one need be described.

50 A valve stem 98 passes through projection 97 and seats at 99, at the end of the projection. This valve is normally held closed by a piston 100 attached to the outer end of the valve stem and normally forced inward by a spring 101.

Air from pipe 95 enters a passage 102 in the mold half, and a branch 103 leads from passage 102 to the passage around each valve stem 98. A screw 104 closes the outer 60 end of branch passage 103, and this screw may be used, if desired, to adjust the size of the opening into the branch passage.

65 Preferably, the end of valve stem 98 is provided with a tip 105 of graphite or similar material, which is refractory and a poor

conductor of heat, and a washer 106 of similar material is applied to the end of projection 97.

In the operation of this device, the mold is operated and the metal is introduced into 70 the mold in the same way as described above in connection with mold 19. During this time valve 90 remains closed.

When it is time to discharge the metal from the interior of the casting, valve 90 is 75 opened, and compressed air, passing through pipe 95 and passageways 102 and 103, presses pistons 100 outward and so opens the inlet passages at valve seats 99. The air then enters the hollow casting and expels the 80 molten metal therefrom without the necessity for the passage of gas through the molten metal.

Graphite tip 105 and washer 106 are used so that little, if any, metal solidifies at this 85 point, and the air has a practically free passage into the interior of the casting, but if the tip and washer are omitted, pressure sufficient to puncture the shell can be used, as the shell will be thinner over such a projection than elsewhere, even if of the same material.

The article produced in this mold is a hollow head 107, such as shown in Fig. 12, having a hole 108 in each ear, through which 95 the metal-expelling air enters. Obviously, other hollow articles, having more than one opening into the interior, may be constructed in a similar manner by molds of such design that metal may be introduced and expelled 100 through one opening and expelling gas may be introduced through one or more of the other openings. This is a simple and efficient way of introducing the gas, where the casting has more than one opening. Gas 105 introduced in this manner may be heated to some extent, if desired, but not as conveniently as where the gas is introduced through the molten metal, as described in connection with the preferred form.

110 While I have described my invention in connection with the formation of metal articles and, for convenience, use the term "metal" in the claims, it will be readily understood that my invention is applicable to substances other than those commonly classified as metals, where the physical characteristics of the substances are such that the features of the invention are applicable thereto for the purposes described.

115 It will be understood that different shapes of articles may be produced by my apparatus and process, and that many changes, not specifically enumerated, may be made within the scope of the appended claims which define my invention.

120 What I claim is:

1. A method of forming hollow metal articles, which consists in filling a mold with molten metal, allowing the metal in contact 130

- with the mold to solidify and form a hollow shell, and introducing gas under more than atmospheric pressure into the interior of the shell and emptying molten metal from the 5 shell.
2. A method of forming hollow metal articles, which consists in filling a mold with molten metal, allowing a shell of solidified metal to form against the interior of the 10 mold, and introducing gas under pressure and forcing the liquid metal out of the interior of the shell.
3. A method of forming hollow metal articles, which consists in filling a mold with 15 molten metal through an inlet in its under side, allowing the metal in contact with the mold to solidify and form a hollow shell, and introducing gas through the inlet into the interior of the shell so that it first contacts 20 the molten metal at a point above the inlet, and emptying molten metal from the shell.
4. A method of forming hollow metal articles, which consists in filling a mold with molten metal through an inlet in its under 25 side, allowing the metal in contact with the mold to solidify and form a hollow shell, and introducing gas under pressure through the inlet and forcing out the liquid metal from the shell.
- 30 5. A method of forming hollow metal articles, which consists in filling a mold with molten metal through an inlet in its under side, allowing the metal in contact with the mold to solidify and form a hollow shell, and 35 introducing gas under pressure into the shell at a point above the inlet and displacing the molten metal within the shell.
6. A method of forming hollow metal articles, which consists in filling a mold with 40 molten metal, allowing the metal in contact with the mold to solidify and form a hollow shell, and introducing heated gas under pressure into the interior of the shell and forcing molten metal out of the shell.
- 45 7. A method of forming hollow metal articles which consists in filling a mold with molten metal through an inlet in its bottom, allowing the metal in contact with the mold to solidify and form a hollow shell, and introducing gas through a pipe surrounded 50 by molten metal into the interior of the shell and displacing the molten metal from the shell.
- 55 8. A method of forming hollow metal articles, which consists in filling a mold with molten metal through an inlet in its under side, allowing the metal in contact with the mold to solidify and form a hollow shell, and introducing heated air under pressure 60 into the shell at a point above the inlet and forcing the molten metal from the interior of the shell.
- 65 9. A method of forming hollow metal articles, which consists in filling a mold with molten metal, allowing the metal in contact 70 with the mold to solidify and form a hollow shell, and introducing gas heated to substantially the temperature of the molten metal into the shell and emptying molten metal from the shell.
10. A method of forming a hollow metal article having a single opening, which consists in filling a mold with molten metal, allowing the metal in contact with the mold to solidify and form a hollow shell 75 complete except where the metal enters, and introducing into the interior of the shell a gas so that it first contacts the molten metal at a point within the shell and emptying molten metal from the shell.
11. A method of forming molten metal articles, which consists in filling a mold with molten metal, allowing the metal in contact with the mold to solidify and form a hollow shell, and introducing into the interior of the shell 80 a gas heated to approximately the temperature of the molten metal and which does not re-act injuriously with the molten metal and emptying the shell of molten metal.
12. A method of forming hollow metal 85 articles, which consists in filling a mold with molten metal through an inlet in its under side, allowing the metal in contact with the mold to solidify and form a hollow shell, and introducing into the shell at a point above 90 its inlet a heated gas under pressure which does not re-act injuriously with the molten metal and driving the molten metal out of the shell.
13. A method of forming hollow metal 95 articles, which consists in exhausting the air from a mold, filling the mold with molten metal, allowing the metal in contact with the mold to solidify and form a hollow shell, and introducing into the interior of the shell 100 a gas under pressure and forcing molten metal from the shell.
14. A method of forming hollow metal 105 articles, which consists in exhausting the air from a mold, filling the mold with molten metal through an inlet in its under side, allowing the metal in contact with the mold to solidify and form a hollow shell, and introducing gas into the shell so that 110 it first contacts the molten metal at a point above the inlet and emptying molten metal from the shell.
15. A method of forming hollow metal 115 articles, which consists in exhausting the air from a mold, filling the mold with molten metal through an inlet in its under side, allowing the metal in contact with the mold to solidify and form a hollow shell, and introducing gas under pressure into the shell 120 at a point above the inlet and forcing molten metal out of the shell.
16. A method of forming hollow metal 125 articles, which consists in filling a mold with molten metal through an inlet in its under side, allowing the metal in contact with the 130

mold to solidify and form a hollow shell, and introducing into the interior of the shell gas heated to approximately the temperature of the molten metal, and emptying molten metal from the shell.

17. A method of forming hollow metal articles, which consists in positioning a mold so that its inlet is on its under side, dipping the inlet into a bath of molten metal, exhausting the air from the mold and filling the mold with molten metal, allowing the metal in contact with the mold to solidify and form a hollow shell, and introducing gas into the shell and emptying molten metal from the shell back into the bath.

18. A method of forming hollow metal articles, which consists in positioning a mold with its inlet on its under side, dipping the inlet in a bath of molten metal, exhausting the air from the mold and filling the mold with molten metal, allowing the metal in contact with the mold to solidify and form a hollow shell, and introducing compressed gas into the interior of the shell at a point above the inlet and forcing molten metal out of the shell.

19. A method of forming hollow metal articles, which consists in filling a mold with molten metal, allowing the metal in contact with the mold to solidify and form a hollow shell, introducing gas into the interior of the shell and emptying molten metal from the shell, and governing the thickness of the shell by the rapidity of cooling of the metal in contact therewith.

20. A method of forming hollow metal articles, which consists in filling a mold with molten metal, allowing the metal in contact with the mold to solidify and form a hollow shell, introducing gas into the interior of the shell and emptying molten metal from the shell, and regulating the temperature of the mold to govern the thickness of the shell.

21. A method of forming hollow metal articles, which consists in filling a mold with molten metal, allowing the metal in contact with the mold to solidify and form a hollow shell, introducing gas into the interior of the shell and emptying molten metal from the shell, and regulating the temperature of the molten metal to govern the thickness of the shell.

22. A method of forming hollow metal articles, which consists in filling a mold with molten metal, allowing the metal in contact with the mold to solidify and form a hollow shell, introducing gas into the interior of the shell and emptying molten metal from the shell, and regulating the temperature of the introduced gas to govern the thickness of the shell.

23. A method of forming hollow metal articles, which consists in filling a mold with molten metal through an inlet, allowing the metal in contact with the mold to solidify

and form a hollow shell, introducing gas under pressure into the interior of the shell and forcing molten metal out of the shell through said inlet, and regulating the pressure of the gas to govern the relative thickness of the shell adjacent the inlet.

24. A method of forming hollow metal articles, which consists in positioning a mold with its inlet downward, dipping the inlet into molten metal, exhausting the air from the interior of the mold and filling the mold with molten metal, allowing the metal in contact with the mold to solidify and form a hollow shell, introducing gas under pressure into the interior of the shell above the inlet, and forcing the molten metal out of the shell and regulating the pressure of the gas to govern the relative thickness of the shell adjacent the inlet.

25. The method of forming hollow metal articles, which consists in positioning a mold with its inlet downward, dipping the inlet into a bath of molten metal, exhausting the air from the mold and filling the mold with molten metal, allowing the metal in contact with the mold to solidify and form a hollow shell, introducing gas into the interior of the shell and emptying out molten metal from the shell while holding the mold in such a position that all its interior surfaces are at an angle to the horizontal.

26. The method of forming hollow metal articles, which consists in positioning a mold with its inlet downward, dipping the inlet into a bath of molten metal, exhausting the air from the mold and filling the mold with molten metal, allowing the metal in contact with the mold to solidify and form a hollow shell, introducing gas through the bath into the interior of the shell and emptying molten metal from the shell.

27. The method of forming hollow metal articles, which consists in positioning a mold with its inlet downward, dipping the inlet into a bath of molten metal, exhausting the air from the mold and filling the mold with molten metal, allowing the metal in contact with the mold to solidify and form a hollow shell, introducing gas through the bath into the interior of the shell and emptying molten metal from the shell while holding the mold in such a position that all of its interior surfaces are at an angle to the horizontal.

28. A method of forming hollow metal articles, which consists in filling a mold with molten metal, allowing the metal in contact with the mold to solidify and form a hollow shell, introducing gas into the interior of the shell and emptying molten metal from the shell and thereafter introducing gas under pressure into the shell within the mold.

29. The method of forming hollow metal articles, which consists in positioning a mold with its inlet downward, dipping the inlet into a bath of molten metal, exhausting the

air from the mold and filling it with molten metal, allowing the metal in contact with the mold to solidify and form a hollow shell, introducing air under pressure into the shell, 5 emptying molten metal from the shell, and thereafter subjecting the interior of the shell within the mold to gas under pressure.

30. The method of forming hollow metal articles, which consists in positioning a mold 10 with its inlet downward, dipping the inlet into a bath of molten metal, exhausting the air from the mold and filling it with molten metal, allowing the metal in contact with the mold to solidify and form a hollow shell, 15 introducing gas through the bath into the interior of the shell and emptying molten metal from the shell, and thereafter subjecting the interior of the shell to gas under pressure.

20 31. The method of forming hollow metal articles, which consists in positioning a mold with its inlet downward, dipping the inlet into a bath of molten metal, exhausting the air from the mold and filling it with molten 25 metal, allowing the metal in contact with the mold to solidify and form a hollow shell, introducing gas through the bath into the interior of the shell and emptying molten metal from the shell while holding the mold 30 in such a position that all of its interior surfaces are at an angle to the horizontal, and thereafter subjecting the interior of the shell to gas under pressure.

32. Apparatus for forming hollow metal 35 articles comprising a mold, means to fill the mold with molten metal, and means to introduce gas under pressure into the interior of the mold to drive out unsolidified portions of the molten metal.

40 33. Apparatus for forming hollow metal articles comprising a mold, means for filling the mold with molten metal, means for introducing gas into the mold to displace therefrom unsolidified molten metal, and 45 means for subjecting the interior of a hollow shell thus formed within the mold to gas under pressure.

34. Apparatus for forming hollow metal articles comprising a mold, means to position the mold with its inlet downward, means to fill the mold with molten metal through its inlet, and a pipe in position to introduce gas through the central portion of the inlet into the interior of the mold cavity 55 to displace the molten metal therefrom.

35. Apparatus for forming hollow metal articles comprising a mold, means to position the mold with its inlet downward, means to fill the mold with molten metal through 60 its inlet, and a gas pipe passing through the inlet and opening into the interior of the mold cavity at a point near the top of the mold cavity.

36. Apparatus for forming hollow metal 65 articles comprising a mold, a receptacle

adapted to contain a bath of molten metal, means to move the mold into position with its inlet dipped into a bath within said receptacle, and a gas pipe extending through said receptacle and through the inlet of the mold when the mold is so positioned. 70

37. Apparatus for forming hollow metal articles comprising a mold, a receptacle adapted to contain a bath of molten metal, 75 means to move the mold into position with its inlet dipped into a bath within said receptacle, a gas pipe extending through said receptacle and through the inlet of the mold when the mold is so positioned, means to exhaust air from the interior of the mold, and 80 means to introduce gas through said gas pipe into the interior of the mold.

38. Apparatus for forming hollow metal articles comprising a mold, a receptacle adapted to contain a bath of molten metal, 85 means to move the mold into position with its inlet dipped into a bath within said receptacle, a gas pipe extending through said receptacle and through the inlet of the mold when the mold is so positioned, means to exhaust air from the interior of the mold, 90 means to introduce gas through said gas pipe into the interior of the mold, and a valve in the end of the gas pipe within the mold.

39. Apparatus for forming hollow metal 95 articles comprising a mold, a receptacle adapted to contain a bath of molten metal, means to position the mold with its inlet in a bath within the receptacle, a gas pipe extending through the bath into the mold 100 when so positioned, means to exhaust air from the mold, a valve for admitting compressed gas into said pipe, a valve in the end of said pipe within the mold, and relief means between said valves for reducing the 105 pressure to atmospheric when the said pressure valve is closed.

40. Apparatus for forming hollow metal articles comprising a mold, a receptacle adapted to contain a molten metal bath, 110 means for moving the mold in a fixed path from a position with its inlet dipped in a bath of molten metal within the receptacle to a discharge position, and a blow-head adjacent the path of the inlet of the mold between said two positions. 115

41. Apparatus for forming hollow metal articles comprising a mold, a receptacle adapted to contain a bath of molten metal, means to move a mold from a position with its inlet dipped in the bath to a discharge position, means to exhaust air from the interior of the mold, means to introduce gas into the interior of the mold to displace molten metal therefrom, and a blow-head 120 adjacent the path of the mold inlet between said two positions. 125

42. Apparatus for forming metal articles comprising a mold, a receptacle adapted to contain a bath of molten metal, means to 130

move the mold between a position with its inlet dipped in a bath of molten metal in the receptacle and a discharge position, a handle adapted to open and close the mold, a 5 vacuum valve for the mold and operative connections between said handle and valve.

43. Apparatus for forming metal articles comprising a mold, a receptacle adapted to contain a bath of molten metal, means to 10 move the mold between a position with its inlet dipped in a bath of molten metal in

the receptacle and a discharge position, a handle adapted to open and close the mold, a vacuum valve for the mold and operative connections between said handle and valve, 15 said operative connections being constructed to operate by additional movement of said handle after the mold is closed and before it is opened.

In testimony whereof, I have hereunto signed my name to this specification.

AUGUST KADOW.